# EUROPEAN PATENT SPECIFICATION

(11) **EP 0 024 217 B1**
(45) Date of publication and mention of the grant of the patent: **11.07.1984**
(21) Application number: 80302885.1
(22) Date of filing: 20.08.1980
(51) Int. Cl.: C22C 33/02, C22C 38/16, B22F 3/12

(54) **Process for producing a compacted powder metal part**
Verfahren zur Herstellung eines Presskörpers aus Metallpulver
Procédé de fabrication d'une pièce compactée à partir de poudre métallique

(30) Priority: 20.08.1979 US 68248
(43) Date of publication of application: 25.02.1981
(73) Proprietor: PITNEY BOWES, INC., Stamford Connecticut 06926 (US)
(72) Inventor: Chen, Yew-Tsung, Trumbull Connecticut 06611 (US)
(74) Representative: Cook, Anthony John

## Description

This invention relates to a process for producing compacted powder metal parts from an Fe-Ni-Mn-Mo powder composition.

Many commercial powder metals are available for fabrication of metal parts by compacting, sintering, and heat treating. One of the more frequently used and readily available metal powders is manufactured and marketed by Hoeganaes Corp. of U.S.A. under the trade name 'Ancorsteel 4600V'. Although this metal powder when used in the fabrication of parts has shown good results, it has certain shortcomings which would be advantageous to eliminate. The specific composition of Ancorsteel 4600V is 1.8% Ni, 0.25% Mn, 0.5% Mo and the balance being Fe. This composition with appropriate amounts of carbon and zinc stearate will hereinafter be referred to as the known composition. It has been found that using this composition results in too much shrinkage during the sintering stage and the parts are generally difficult to machine. Obviously, it would be advantageous if these shortcomings could be eliminated without sacrificing the generally high strength and ductility possessed in parts made from such a metal powder composition.

In accordance with the present invention, it has been found unusually advantageous to add a small quantity (i.e. 0.5 to 1.5% by weight) of copper to the known composition when metal parts are to be fabricated. Including the small quantity of copper to the known composition and processing parts made from these compositions in accordance with the process described hereinbelow has not only resulted in better machinability and reduction of shrinkage of the parts, but surprisingly has yielded parts with higher tensile strengths and higher toughness. The known composition having a small amount of copper added thereto will hereinafter be referred to as the disclosed composition. Furthermore, all percent composition figures mentioned herein are percent by weight unless stated otherwise.

In accordance with this invention, there is provided a process for producing a powder metal part comprising the steps of compacting a powder metal composition comprising 1.0-2.5% Ni, 0.3-0.7% Mo, 0.15-0.30% Mn, 0.5-1.5% Cu, 0.3-0.7% C, 0.5-1.0% zinc stearate, the balance being Fe, the compaction being under sufficient pressure to form a part having a density ranging from 6.4 g/cm³ to 7.1 g/cm³; and sintering the compressed part at a temperature ranging from 2000°F (1093°C) to 2150°F (1177°C) for 15 to 30 minutes in a furnace having a dew point ranging from 20°F (-6.7°C) to 61 °F (16°C) and under an endothermic atmosphere.

A sintering temperature of 2050°F (1120°C) with a dew point of 30-55°F (-1 to +7°C) has been found to be very well suited for this process. Although many of the known endothermic type atmospheres can be used, it has been found that an atmosphere comprising nitrogen, hydrogen and carbon monoxide is preferred.

The copper content is preferably substantially 0.75-1.0%. The carbon content is preferably 0.45-0.55%. The part may be cooled after sintering substantially at a cooling rate of 1.5 to 10°F (1 to 5.5°C) per second. The compaction step may be carried out substantially at a pressure in the range of 28 to 50 t.s.i. (440xl 0⁶ to 784x 1 0⁶ Pa).

Preferred embodiments of the invention will now be described.

It has been found that adding an amount in the range 0.5-1.5% copper to known metal powder mixtures of 1.0-2.5% Ni, 0.15-0.30% Mn, 0.3-0.7% Mo, 0.3-0.7% C and 0.5-1.0% zinc stearate, the balance being iron, has resulted in a metal powder which, when compacted, sintered and heat treated, results in a metal part having unusually and surprisingly good properties. This is particularly true of the metal part that results from the sintering stage. As is known, it is advantageous to have a sintered piece with high strength as the same may be subjected to stresses during the heat treat stage.

In adding the copper to the known composition and sintering in accordance with the process described herein, it was found that the tensile strength increased after heat treating and the fracture toughness increased after heat treating. With regard to machinability, it was found that drill bits used to machine the heat treated products made in accordance with this invention lasted from 50-100% longer than those used to machine products made in like manner but from the known composition.

### Example 1 (State of the art according to Rule 54(3)

A composition was prepared having, by weight, the following ingredients:

A 1.25"×0.5"×.25" (31.75×12.7×6.35 mm) transverse rupture bar was compacted at 50 tsi (tons per square inch) 784x 10⁶ Pa and sintered at 2050°F (1120°C) for 15-30 minutes, with a dew point of 35°-55°F (1.7 to 13°C) and under endothermic atmosphere. There was only 0.0006" (0.015 mm) shrinkage in length. After carbonitriding at 1550°F (843°C) for 30 minutes, the bar was oil quenched and tempered at 350°F (177°C) for one hour. There was only 0.0008" (0.02 mm) expansion.

In addition to maintaining stable dimensions, high strength and toughness was also achieved.

A number of samples having the above dimensions from both the known and the disclosed compositions were made by the process described above. In one series of tests the percentages of ingredients (except copper) as stated above were kept constant and the amount of copper was varied from 0.77 to 1.22%. In another series of tests the percentages of ingredients (except carbon) were kept constant as stated above and the carbon content was varied from 0.35 to 0.55%. All such samples of the disclosed composition were found to give superior results.

The samples of the disclosed composition resulting from Example I were found to have a transverse rupture strength of approximately 160,000 psi (1103 M Pa) after sintering and a transverse rupture strength of approximately 200,000 psi (1379 M Pa) after heat treating. This compares with a transverse rupture strength of approximately 141,000 psi (1034 M Pa) for the known composition in the sintered condition and approximately 196,000 psi (1351 M Pa) in the heated treated condition. The disclosed composition was found to have a fracture toughness as sintered of approximately 21,000 psi-in^{1/2} (23.1 M Pa-m.^{1/2}) and 23,000 psi-in"2 (25.3 M Pa-m.^{1/2}) in the heat treated condition. This compares with the known composition having a sintered fractured toughness of approximately 21,000 psi-in^{1/2} (23.1 M Pa-m^{1/2}) both in the sintered and heat treated condition.

With respect to machinability, a test was run wherein a drill bit with a load of 24 lbs. (10.89 kg) was applied to the above samples and rotated at a speed of 1,000 RPM. These loads were applied to samples which had a thickness of approximately 1/4" (6.35 mm). For the disclosed composition it was found that approximately 11 seconds were required to drill through a sample and for the known composition approximately 15 seconds were required. Even more significant was that the drill bit showed considerably more wear after drilling through the known composition than it did after drilling through the disclosed composition.

The tensile strengths of samples made from the disclosed composition were measured and found to be 81,000 psi (558.5 N per sq. mm) sintered and 125,000 psi (861.9 N per sq. mm) heat treated whereas samples made from the known composition were found to be 75,000 psi and 110,000 psi (517.1 and 758.5 N per sq. mm) respectively.

### Example II

A composition was prepared having, by weight, the following ingredients:

The above composition was compacted as tollows:

The composition was sintered in a moving belt sintering furnace under the following conditions:

The properties of the sintered composition were as follows:

When parts formed of the Ancorsteel 4600V alloy with 0.45% carbon (known composition) was sintered by the process described herein the following properties were observed.

### Example III

A composition was prepared having, by weight, the following ingredients:

The above composition was compacted as follows:

The composition was sintered in a moving belt sintering furnace under the following conditions.

The properties of the sintered composition were as follows:

It will be seen from the foregoing disclosure that substantially better results are achieved by making parts using the composition having 0.5-1.5% of copper added thereto, and by employing the sintering process as disclosed. These findings have been unexpected and gratifying, in that desirable increased physical properties have been obtained without undue complexity or expense of processing.

A process which operates according to the parameters stated in Example I herein has been disclosed in the European Patent Application No. 79302280.7 (Publication No. 10442), and is claimed in the divisional European Patent Application No. 81200710.2 (Publication No. 42200) and, in this patent application, no claim is made to the subject matter of Example I. Subject to this disclaimer, what is claimed herein is as follows.

## Claims

1. A process for producing a powder metal part comprising the steps of compacting a powder metal composition comprising 1.0-2.5% Ni, 0.3-0.7% Mo, 0.15-0.30% Mn, 0.5-1.5% Cu, 0.3-0.7% C, 0.5-1.0% zinc stearate, the balance being Fe, the compaction being under sufficient pressure to form a part having a density ranging from about 6.4 g/cm³ to 7.1 g/cm³; and sintering the compressed part at a temperature ranging from 2000°F (1093°C) to 2150°F (1177°C) for 15 to 30 minutes in a furnace having a dew point ranging from 20°F (-6.7°C) to 61 °F (16°C) and under an endothermic atmosphere.

2. A process according to claim 1 in which the dew point is in the range 30°F (-1 °C) to 35°F (2°C).

3. A process according to claim 1 or 2 in which said endothermic atmosphere is formed of a gas comprising nitrogen, hydrogen and carbon monoxide.

4. A process according to any preceding claim in which the part is cooled after sintering at a cooling rate of 1.2 to 10°F per second (0.67°C to 5.6°C per second).

5. A process according to any preceding claim in which the compaction step is carried out at a pressure in the range 440x10⁶ to 784×10⁶ Pa (28-50 tsi).

6. A process according to any preceding claim in which the compacted metal powder part has a density substantially in the range 6.5 to 7.03 grams per cm³.

## Patentansprüche

1. Verfahren zur Herstellung eines Pulvermetallteiles mit den Stufen eines Pressens von Metallpulver aus 1,0 bis 2,5% Ni, 0,3 bis 0,7% Mo, 0,15 bis 0,30% Mn, 0,5 bis 1,5% Cu, 0,3 bis 0,7% C, 0,5 bis 1,0% Zinkstearat und Rest Fe, wobei das Pressen unter einem ausreichenden Druck erfolgt, um ein Teil mit einer Dichte im Bereich von etwa 6,4 g/cm³ bis etwa 7,1 g/cm³ zu bilden, sowie eines Sinterns des gepreßten Teils bei einer Temperatur im Bereich von etwa 2.000°F (1.093°C) bis etwa 2.150°F (1.177°C) während etwa 15 bis etwa 30 Minuten in einem Ofen mit einem Taupunkt im Bereich von etwa 20°F (-6,7°C) bis etwa 61 °F (16°C) und unter einer endothermen Atmosphäre.

2. Verfahren nach Anspruch 1, in dem der Taupunkt im Bereich von 30°F (-1 °C) bis 35°F (2°C) liegt.

3. Verfahren nach Anspruch 1 oder 2, in welchem die endotherme Atmosphäre von einem Gas gebildet wird, das Stickstoff, Wasserstoff und Kohlenmonoxid umfaßt.

4. Verfahren nach einem der vorausgehenden Ansprüche, in welchem das Teil nach dem Sintern im wesentlichen mit einer Kühlgeschwindigkeit von 1,2 bis 10°C/sec (0,67°C bis 5,6°C/sec) gekühlt wird.

5. Verfahren nach einem der vorausgehenden Ansprüche, in welchem die Preßstufe bei einem Druck im Bereich von 440x 10⁶ bis 784x10⁶ Pa (28 bis 50 tsi) durchgeführt wird.

6. Verfahren nach einem der vorausgehenden Ansprüche, in welchem das gepreßte Metallpulverteil eine Dichte im wesentlichen im Bereich von 6,5 bis 7,0 g/cm³ besitzt.

## Revendications

1. Procédé pour produire une pièce en métal pulvérulent, caractérisé en ce qu'il comprend les étapes de tasement d'une composition métallique pulvérulente comprenant 1,0 à 2,5% de Ni, 0,3 à 0,7% de Mo, 0,15 à 0,30% de Mn, 0,5 à 1,5% de Cu, 0,3 à 0,7% de C, 0,5 à 1,0% de stéarate de zinc, le reste étant constitué par du Fe, le tassement étant réalisé sous une pression suffisante pour former une pièce ayant une densité dans la gamme d'environ 6,4 g/cm³ à 7,1 g/cm³, et de frittage de la pièce tassée à une température allant d'environ 1093°C (2000°F) à environ 1177°C (2150°F) pendant environ 15 à 30 minutes, dans un four ayant un point de rosée dans la gamme d'environ -6,7°C (20°F) à 16°C (61°F) et sous une atmosphère endothermique.

2. Procédé selon la revendication 1, caractérisé en ce que le point de rosée est dans la gamme de -1°C (30°F) à 2°C (35°F).

3. Procédé selon l'une quelconque des revendications 1 ou 2, caractérisé en ce que l'atmosphère endothermique est formée d'un gaz comprenant de l'azote, de l'hydrogène et du monoxyde de carbone.

4. Procédé selon l'une quelconque des revendications précédentes, caractérisé en ce qu'après la frittage, on refroidit la pièce pratiquement avec une vitesse de refroidissement de 0,67°C à 5,6°C par seconde (1,2'à à 10°F par seconde).

5. Procédé selon l'une quelconque des revendications précédentes, caractérisé en ce que l'on réalise l'étape de tassement à une pression dans la gamme de 440.106 à 784.106 Pa (28-50 tsi).

6. Procédé selon l'une quelconque des revendications précédentes, caractérisé en ce que la pièce en poudre métallique tassée présente une densité qui est pratiquement dans la gamme de 6,5 à 7,03 grammes par cm³.
